

## UNITED STATES PATENT OFFICE

2,171,249

CATHODE FOR ELECTRON DISCHARGE  
DEVICES

Erich Wiegand, Berlin-Waidmannslust, Germany,  
assignor to Allgemeine Elektricitäts Gesell-  
schaft, Berlin, Germany, a corporation of Ger-  
many

No Drawing. Application June 14, 1935, Serial  
No. 26,639. In Germany July 11, 1934

5 Claims. (Cl. 250—27.5)

My invention relates to electron discharge de-  
vices and more particularly to oxide coated cath-  
odes for such devices.

During operation of thermionic cathodes in  
5 electron discharge devices, heating energy losses  
caused by radiation may be decreased by using  
for the emitting coatings and the supports there-  
for materials the radiation from which is small  
at the operating temperatures.

10 Particularly suitable for supporting metals are  
gold, silver, or copper, and alloys thereof. While  
nickel has a radiation equal to about 15% of a  
black body, the radiation from copper amounts  
to only about 4%. An indirectly heated equi-  
15 potential cathode of conventional construction  
comprising a metal sleeve and an electron emis-  
sive coating of an alkaline-earth metal oxide, if  
nickel is used for the sleeve, consumes about four  
watts of heating energy, while the same cathode  
20 with a copper sleeve consumes only two watts.  
Cathodes of copper, silver, or gold that is, metals  
of Group 1 Sub 2 of the Periodic table however,  
vary in their emissivities, and they are unsatisfac-  
tory so far as their actual life is concerned.  
25 Oxide cathodes having sleeves of these metals  
usually lose their electron emissivity after a short  
period of time. It is believed that the evolution  
of gases from the metal of the sleeve is respon-  
sible though no conclusive evidence to support  
30 this theory has so far been found.

It is the principal object of my invention to  
provide an improved type of oxide coated therm-  
ionic cathodes.

Oxide coated cathodes with supporting sleeves  
35 consisting of metals of low radiation characteris-  
tics and made according to my invention have  
life and emission characteristics which are sub-  
stantially the equivalent to cathodes made from  
nickel or platinum. According to my invention  
40 instead of pure metals, such as nickel, I use cop-  
per, silver, or gold, or alloys thereof, which apart  
from the chief metal of lower total radiation, con-  
tain a small amount of certain other metals.  
45 For example, particularly favorable results are  
obtained with sleeves or sheaths which consist  
of an alloy composed roughly of from 99.9% to  
95% copper and of from 0.1 to 5% nickel. A sim-  
ilar action is exhibited also by iron, cobalt, plati-  
num, iridium, osmium, ruthenium, rhodium and  
50 palladium, in other words, all metals belonging  
to the eighth group of the periodic system of the  
elements which are capable of being alloyed with  
copper, silver, and gold.

It is preferable not to choose a mixture such  
55 that the favorable radiation properties of the

main metal are lost as a consequence. The radia-  
tion characteristic of the alloys of copper, silver  
and gold with the other above mentioned metals  
differ only slightly from the radiation character-  
istics of the unalloyed metal as long as the mix-  
ture does not exceed a certain limit. This limit is  
not the same for the various additional metals  
for a given metal. As a general rule, however,  
alloys which contain over 10% of the additional  
metal, are not quite so favorable in their radia-  
tion characteristics, although the long life of the  
cathodes made in accordance with my invention  
are preserved.

5 The cathodes made of alloys of the kind sug-  
gested may be made in various ways. As pure  
metals as are obtainable should be used, for in-  
stance, electrolytic copper and nickel made from  
nickel carbonyl, and the alloy should be made in  
vacuo or in the presence of gases of a nature  
10 which will not be converted with constituents  
of the alloys. The alloys can be made in the usual  
way from the pure metals by melting, and may  
thereupon be worked into ribbons, wires, tubes or  
sleeves. However, it is also practical to first make  
15 ribbons, wires or tubes of the pure main metals  
and then coat them, say by an electrolytic proc-  
ess, with the added metal, and to finally insure  
formation of the alloy in the finished cathode  
sleeve or core by tempering. It is even practical  
20 to cause formation of the alloy after application  
of the electron emitting coatings and the cathode  
has been placed in the tube either during or after  
the exhausting of the tube, for example, during the  
forming or activating process. It is suitable to  
25 cause the alloying prior to the use of the tube  
to a point where its characteristics have become  
stable. In some instances the alloying improves  
during the life of the tube and the reduction in  
30 electron emissivity which is occasionally observed  
in long life cathodes will not take place because  
of the increase in working temperature of cath-  
odes made in accordance with my invention.

35 Using copper as the main metal it may, under  
certain circumstances, be advantageous to incor-  
porate in the alloy small quantities, up to about  
1%, of a de-oxidizing agent such as calcium, sili-  
40 cium, or calcium boride, with the result that such  
small quantities of oxygen as may have gotten  
into the alloy during working are made ineffec-  
tive.

45 It is not necessary that the entire cathode sup-  
port should be coated with the added or ad-  
ditional metal. For example, such portions of the  
cathode as stay cold in operation may be left  
50 unalloyed.

5

10

20

25

30

35

40

45

50

55

As a general rule, the electron emitting coatings, such as coats of alkali-earth metal oxides, should not be thicker than 100 microns lest the low radiation of the supporting metal wire or sleeve be partly offset by the high radiation of the oxide coating.

With a view to reducing the heat losses it is advantageous in practice to make the current leads from materials having inherently low heat 10 conducting powers.

While the applicant is not to be limited to any particular theory, it is believed that the main metals, after alloying, no longer absorb certain gases which disturb the electron emission or yield them during the operation of the cathode. It may also be that the additional metals tend to increase the adhesiveness of the electron emitting-coats. Compared with pure copper, alloys of copper with the metals indicated show also a substantially greater stability towards atmospheric agencies; and this fact is of considerable importance so far as the method of manufacturing thermionic cathodes is concerned.

While I have indicated the preferred embodiments of my invention of which I am now aware and have also indicated only one specific application for which my invention may be employed, it will be apparent that my invention is by no means limited to the exact forms illustrated or the use indicated, but that many variations may be made in the particular structure used and the purpose for which it is employed without departing from the scope of my invention as set forth in the appended claims.

What I claim as new is:

1. In an electron discharge device, a cathode support having an oxide coating and comprising an alloy of only a metal of Group 1 Sub 2 of the periodic table and a metal of the eighth group 5 of the periodic system comprising not more than 10% of the alloy.

2. In an electron discharge device, a cathode support having an oxide coating and comprising an alloy including only copper and a metal of 10 the eighth group of the periodic system of the elements, said metal comprising not more than 10% of the alloy.

3. In an electron discharge device, a thermionic cathode of the oxide coated type including a 15 support for the oxide coating formed of an alloy containing only copper and up to 10% of a metal of the eighth group of the periodic system and up to 1% of a deoxidizing agent.

4. In an electron discharge device, a thermionic 20 cathode of the oxide coated type including a supporting base of only copper of not less than 95% of the total and nickel of not more than 5% of the total.

5. In an electron discharge device, a thermionic 25 cathode of the oxide coated type including a supporting base of only copper of not less than 95% of the total and nickel of not more than 5% of the total, and a deoxidizing agent up to 1%.

ERICH WIEGAND. 30